

1

3,179,592  
LUBRICANT CONTAINING BIS(TRI-CHLOROMETHYL)BENZENE

Robert K. Smith and Paul J. Welsh, Springfield Township, Pa., assignors to Diamond Alkali Company, Cleveland, Ohio, a corporation of Delaware  
No Drawing. Filed Mar. 20, 1963, Ser. No. 266,522  
11 Claims. (Cl. 252—58)

This invention relates to an improved extreme pressure agent and to a lubricant containing it. More particularly, this invention concerns an oil-soluble additive material capable of imparting extreme pressure, increased load carrying capacity and anti-wear properties to lubricating oils without upsetting other desired characteristics of the lubricant.

It is well known that the high pressure occurring in certain types of gears and bearings may cause a film of lubricant to rupture with consequent damage to the machinery. It has been shown that base lubricants such as mineral oil and/or synthetic oil can be improved with regard to their protective effect, particularly on rubbing surfaces by the addition of certain substances, so that excessive wear, scuffing and seizure, which normally follow a break in the film of the lubricant, can be prevented even under very unfavorable pressure and speed conditions. Lubricants possessing the highly desirable property are called extreme pressure lubricants.

Extreme pressure lubricants have found extensive use as gear lubricating fluids, such as in the lubrication of gear differentials of trucks and other vehicles. The lubrication of gears demands lubricants of special qualities particularly high lubricity and high film strength. When a lubricant is compressed between two moving metallic surfaces, high film strength is necessary to prevent direct metal-to-metal contact of said surfaces, with consequent welding. The extreme pressures to which lubricants are subjected when compressed between hypoid gear surfaces cause a rise in internal heat which is augmented by any heat from friction generated by lack of point-lubricity. It has been found that oleaginous liquid lubricant bases such as mineral lubricating oils, esters, whether natural esters, for example, castor oil or sperm oil or synthetic ester lubricants and other synthetic lubricants alone are unsatisfactory in that they do not have the required high lubricity and high film strength and consequently allow scoring and welding of gears on continued use.

Many types of additives have been prepared and added to extreme pressure lubricant formulations for the purpose of augmenting film strength, lubricity and other desired characteristics. Fatty oils and fatty acid esters, for example, have been added in various amounts and combinations to hydrocarbon oil fractions, particularly for the purpose of furnishing "oiliness," that is to say, high lubricity. It has also been found that when sulfur-containing compounds are added to extreme pressure lubricants, film strength is somewhat increased, and recent formulations have combined ester additives with sulfur by sulfurizing said esters to provide both lubricity and film strength of high degree. Still more recently, it has been discovered that the use of phosphorus in combination with the sulfur-containing ester additives has further augmented desired film strength to a level of highly satisfactory performance. Thus, oils and fatty esters may have incorporated therein phosphorus and sulfur by reaction with any one of a number of phosphorus sulfide compounds, such as phosphorus sesquioxide. The increased performance of phosphorus and

2

sulfur-containing esters as additives for extreme pressure lubricants, when compared with sulfur-containing esters as additives for extreme pressure lubricants, may be seen in that the former are effective for transmissions operating at both low speed and high torque, and at high speed and low torque, whereas esters which have only been sulfurized and which are considered suitable extreme pressure additives exhibit in the extreme pressure lubricants satisfactory performance only under conditions of low speed and high torque.

It has now been discovered that satisfactory extreme pressure and anti-wear lubricants can be obtained by incorporating into a base lubricant aromatic compound possessing the trichloromethyl grouping, i.e.,  $-\text{CCl}_3$ . More particularly, the present invention resides in an extreme pressure lubricating composition comprising a major amount of base lubricating oil and a minor amount sufficient to impart extreme pressure characteristics to the base oil of an additive having the following structural formula:



wherein R is an aromatic hydrocarbon ring, preferably  $\text{C}_6\text{H}_4$ ; —f— indicates a fused ring relationship (two carbon atoms common to two aromatic nuclei, e.g., as in naphthalene); m is generally 0 to 1 or more; x is an integer of from about 0 to 4 or more, preferably from 0 to 2 and y is an integer of from about 2 to 6, preferably from 2 to 3. The preferred aromatics, however, include trichloromethylated benzenes corresponding to the above formula when m is 0; x is 0 and y is 2. Such preferred aromatics include, for instance, a,a'-hexachloro-p-xylene; a,a' - hexachloro-m-xylene; a,a'-hexachloro-o-xylene and mixtures of such isomers.

The additive is prepared by the photochemical chlorination of the appropriate xylene isomer or mixtures of the same giving the corresponding polychloro derivatives by the replacement by chlorine of the side-chain hydrogen. Such methods are described in French Patent 798,727 and Chemical Abstracts, 49, 14670 f. The preparations of the additive are subject to variation as to the relative amounts of the respective reactants employed. Generally, the chlorine will be employed in a molar excess relative to the xylene, usually in amounts of up to about 8 moles of chlorine per mole of xylene. The reaction is conducted in the presence of any suitable ultra violet light as a source of photoactivation such as a mercury vapor lamp, for example, a 360-watt G.E. Uviarc mercury vapor lamp in a single-wall Pyrex well or a 450-watt Hanovia mercury vapor lamp in a double well, with the lower half of each well made of Corex type D glass to transmit ultraviolet wave lengths.

The reaction may be accelerated and/or its course controlled by the application of heat to the reaction mixture. The reaction temperature may vary from about 70° C. to about 150° C. Excessively high temperatures may cause some decomposition and are thereby undesirable. The use of lower temperatures merely reduces the rate of reaction. Temperatures between about 80° C. and about 140° C. are preferred. Usually the reaction temperature is maintained at about 80° C. to 90° C. for about the first three or four moles of reacted chlorine, at which point the reaction temperature is raised and maintained at about 135° C. for the remainder of the reaction.

The time of reaction may vary from about 6 to about 35 or more hours, depending on the temperature employed, with a preferred maximum time of about 30 hours.

Pressure techniques may also be utilized to prepare the extreme pressure additive of the present invention. Pressures are generally maintained in the reaction vessel within the range of about 10 to about 40 p.s.i.g., preferably about 20 to 35 p.s.i.g. The reactants may be micro-filtered in order to remove iron from the raw materials which, if present during the reaction, causes discoloration of the batch, promotes ring chlorination and decomposition and reduces light transmission. Also a sequestering agent may be used to sequester traces of iron which remains in the reactor charge. A suitable sequestering agent includes triphenyl phosphate.

After the reaction is completed, the reaction vessel is swept with an inert gas such as air or nitrogen to render the system substantially free of HCl gas. The product is then dissolved in a solvent such as acetic acid, methanol, ethanol, isopropanol, etc. and cooled to about 20° C. and filtered resulting in a recovery of a substantially pure hexachloroxylene product. The reaction between the chlorine and xylene may be effected in either a batchwise, an intermittent or a continuous manner.

The base oil in our improved extreme pressure lubricant may comprise any petroleum or mineral lubricating oil fraction, for instance, a solvent extracted or solvent refined oil obtained in accordance with conventional methods of solvent refining lubricating oils. Often, lubricating oils have viscosities from about 50 to 1000 or more S.U.S. at 100° F. The base oil may be derived from paraffinic, naphthenic, asphaltic or mixed base crudes, and if desired, a blend of solvent-treated Mid-Continent neutrals and Mid-Continent bright stock may be employed. Also contemplated are ester base lubricants such as the synthetic esters, for example, diesters or complex esters, such as di-2-ethylhexyl sebacate. Aside from the hexachloroxylene additive the base oil is usually the essential balance of the composition. However, the composition may also contain minor amounts of other additive agents such as pour depressors, viscosity index improvers, anti-oxidants, foam inhibitors, etc.

The additives of the present invention have been found effective in the base lubricants in amounts ranging between 45

100

40

35

30

25

20

15

10

5

4

## EXAMPLE 1

To a paraffinic base mineral oil having the following characteristics:

|                  |         |
|------------------|---------|
| Gravity          | 26-28   |
| Vis. @ 100° F.   | 100-110 |
| Flashpoint, ° F. | min 360 |
| Firepoint, ° F.  | 410     |
| Pour point, ° F. | +30     |

is added the extreme pressure additive of the present invention in amounts of 1% and 2% by weight, respectively. The various formulations containing the additive are as follows:

|                                                                                                                       | Percent        |
|-----------------------------------------------------------------------------------------------------------------------|----------------|
| Composition A:<br>Paraffin base mineral oil, 100 SUS @ 100° F.                                                        | 100            |
| Composition B:<br>Paraffin base mineral oil, 100 SUS @ 100° F.<br>a,a'-Hexachloro-p-xylene (M.P. 107-110° C.)         | 99<br>1<br>100 |
| Composition C:<br>Paraffin base mineral oil, 100 SUS @ 100° F.<br>a,a'-Hexachloro-p-xylene (crude, M.P. 102°-105° C.) | 99<br>1<br>100 |
| Composition D:<br>Paraffin base mineral oil, 100 SUS @ 100° F.<br>a,a'-Hexachloro-m-xylene                            | 99<br>74       |
| a,a'-Hexachloro-p-xylene                                                                                              | 15             |
| Phenyl pentachloroethane                                                                                              | 6              |
| a,a,a,a',a'-Pentachloro-o-xylene                                                                                      | 5<br>100       |
| Composition E:<br>Paraffin base mineral oil, 100 SUS @ 100° F.<br>a,a'-Hexachloro-m-xylene                            | 99<br>80       |
| a,a'-Hexachloro-p-xylene                                                                                              | 14             |
| Phenyl pentachloroethane                                                                                              | 3              |
| a,a,a,a',a'-Pentachloro-o-xylene                                                                                      | 3<br>100       |
| Composition F:<br>Paraffin base mineral oil, 100 SUS @ 100° F.<br>a,a'-Hexachloro-p-xylene                            | 99<br>84       |
| a,a'-Hexachloro-m-xylene                                                                                              | 16             |
| Composition G:<br>Paraffin base mineral oil, 100 SUS @ 100° F.<br>a,a'-Hexachloro-p-xylene (107°-110° C.)             | 98<br>2<br>100 |

The results from the extreme pressure tests are given in Table I.

Table I

| Composition                                                                        | A                         |              | B                         |    | C            | D            | E            | F            | G                         |
|------------------------------------------------------------------------------------|---------------------------|--------------|---------------------------|----|--------------|--------------|--------------|--------------|---------------------------|
| Extreme pressure test:<br>4-Ball (weld point, kg.)<br>Falex (failed at load, lbs.) | 90<br><500                |              | 224<br>3,000              |    | 224<br>3,000 | 224<br>3,250 | 224<br>3,250 | 224<br>3,500 |                           |
|                                                                                    | Jaw load (lbs.) v. Torque |              | Jaw load (lbs.) v. Torque |    |              |              |              |              | Jaw load (lbs.) v. Torque |
| Almen                                                                              | 20<br>22                  | 30<br>Failed | 130                       | 20 |              |              |              |              | 130                       |
| Cornell                                                                            |                           |              | 4,500                     | 45 |              |              |              |              | 21                        |

<sup>1</sup> Full load.

about 0.1 to about 10, preferably between about 0.5 to 5, weight percent.

In order that those skilled in the art may more completely understand the present invention and the preferred methods by which the same may be carried into effect, the following specific examples are offered:

A series of formulations containing the extreme pressure agent of the present invention were subjected to well known extreme pressure testing techniques such as, for instance, the Timken, Almen, 4-ball and Cornell test methods, to evaluate the additive's effectiveness in various lubricating media. The results are presented in the following examples.

Using the additive of the present invention in a base mineral oil, the weld point using the Shell 4-ball E.P. test is increased by about 150%. Also, the base oil fails at a load of less than about 500 pounds using the Falex E.P. test, whereas when 1% of the additive is present the composition fails at loads of from about 3000 to about 3500 pounds. Further, using the Almen E.P. test on the base oil containing 1% of the additive a torque reading of 26 at a full load of 30 pounds is obtained and when 2% of the extreme pressure additive is added to the base oil a torque reading of 21 at a full load of 30 pounds is obtained, whereas the base oil without the additive when tested on the Almen E.P. tester gives a torque reading of 30 at a load of 20 pounds and fails at 22 pounds. When

1% of the extreme pressure additive is added to the paraffinic base oil and tested on the E.P. Cornell tester a low torque of 45 at 4500 pounds jaw load is obtained.

## EXAMPLE 2

To a 3% emulsion containing:

|                                                                                                                                                                  | Percent  |
|------------------------------------------------------------------------------------------------------------------------------------------------------------------|----------|
| 2-methyl 2,4-pentanediol                                                                                                                                         | 9.6      |
| Straight chain fatty acid (a tall oil fatty acid—aver. C <sub>18</sub> carbon chain length alkyl carboxylic acid containing unsaturated components):             |          |
| Visc. @ 100° F., SUS                                                                                                                                             | 93       |
| Specific gravity 25/25                                                                                                                                           | 0.9005   |
| Iodine value                                                                                                                                                     | 130-140  |
| Saponification No.                                                                                                                                               | 190-195  |
| Flash point, ° F.                                                                                                                                                | 380      |
| Fire point, ° F.                                                                                                                                                 | 415      |
| Pour point, ° F.                                                                                                                                                 | +37      |
| Paraffinic base oil:                                                                                                                                             | 9.6      |
| Visc. @ 100° F.                                                                                                                                                  | 35-40    |
| Flash point, ° F.                                                                                                                                                | min. 260 |
| Fire point, ° F.                                                                                                                                                 | 300      |
| Pour point, ° F.                                                                                                                                                 | max. +30 |
| Sulfur content                                                                                                                                                   | 0.1      |
| Alox 1516 (amine derivative of an oxidized paraffin wax):                                                                                                        | 14.4     |
| Visc. @ 100° F., SUS                                                                                                                                             | 700      |
| Specific gravity @ 127° F.                                                                                                                                       | 1.04     |
| Pour point, ° F.                                                                                                                                                 | +30      |
| Flash point, ° F.                                                                                                                                                | 220      |
| Sterox AS-1 (adduct of nonyl phenol and 9 mols of ethylene oxide)                                                                                                | 1.9      |
| Water                                                                                                                                                            | 4.7      |
| Condensate:                                                                                                                                                      | 28.9     |
| Diethanolamine                                                                                                                                                   | parts 50 |
| Straight chain naphthenic based fatty acid (Aver. C <sub>18</sub> carbon chain length alkyl carboxylic acid containing unsaturated components): Acid No. 160-180 | parts 50 |
|                                                                                                                                                                  | 28.9     |
|                                                                                                                                                                  | 98       |

is added 2% by weight of a,a'-hexachloro-p-xylene (M.P. 107°-110° C.) and the final mixture tested on the Almen tester.

Table II  
ALMEN E.P. TEST

| Jaw load (lbs.) | Torque |
|-----------------|--------|
| 2               | 5      |
| 4               | 6      |
| 6               | 7      |
| 8               | 9      |
| 10              | 10     |
| 12              | 10     |
| 14              | 10     |
| 16              | 10     |
| 18              | 10     |
| 20              | 11     |
| 22              | 11     |
| 24              | 11     |
| 26              | 12     |
| 28              | 15     |
| 30              | 17     |

The data in Table II show that the additive of the present invention gives a torque reading of 17 at a load of 30 pounds (full load), indicating the composition possesses excellent extreme pressure characteristics for a cutting oil.

## EXAMPLE 3

To the following composition:

|                                                                          | Percent     |
|--------------------------------------------------------------------------|-------------|
| Sulfurized fatty esters of lard oil (10-11% sulfur):                     | 800-900     |
| Visc. @ 100° F., SUS                                                     | 35          |
| Chlorinated paraffin wax (aver. C <sub>20-30</sub> carbon chain length): |             |
| Gravity @ 60° F.                                                         | 23-25       |
| Visc. @ 100° F., SUS                                                     | 4,000       |
| @ 210° F., SUS                                                           | 160-180     |
| Percent chlorine                                                         | 41-43       |
| Saponification No.                                                       | 172         |
| Sulfur, wt. percent                                                      | 0.042       |
| Naphthenic base mineral oil:                                             |             |
| Visc. @ 100° F., SUS                                                     | 100-110     |
| Gravity                                                                  | 21-25.5     |
| Flash point, ° F.                                                        | min. 330    |
| Pour point, ° F.                                                         | max. 0      |
| Pine oil:                                                                |             |
| Gravity @ 68° F.                                                         | 20.5-21.5   |
| Flash point, ° F.                                                        | 172         |
| Naphthenic base mineral oil:                                             |             |
| Visc. @ 100° F., SUS                                                     | 2,150-2,200 |
| @ 210° F., SUS                                                           | 80-90       |
| Gravity                                                                  | 18.6        |
| Flash point, ° F.                                                        | 450         |
| Fire point, ° F.                                                         | 500         |
| Pour point, ° F.                                                         | +15         |
| Sulfur, wt. percent                                                      | 0.28        |

is added 3% by weight of a,a'-hexachloro-p-xylene (M.P. 107°-110° C.) and the final mixture tested on the Almen tester for E.P. characteristic. Also, the above composition is tested for its properties as a cutting coolant by Socony Mobil's tapping test method as described in United States Steel Corporation, National Tube Division's bulletin, copyright 1956 on page DM-61. This test consists essentially in placing a test bar in a vise on a turntable of a drill press and tapping a hole in the test bar with the drill lubricated with the test coolant. A torque arm attached to the turntable actuates a spring scale and reports the torque for each tap. The average torque of 30 runs made with five different taps is recorded and compared with the average torque of a known reference oil. The percent efficiency of the coolant to be tested is the net result. Table III presents comparative data showing the improvements which are obtained with the above-described composition with and without the additive of the present invention.

Table III

|                                          | Almen test          | Tapping efficiency, percent |
|------------------------------------------|---------------------|-----------------------------|
| Composition (without additive)           | Failed at 28 pounds | 83                          |
| Composition +3% a,a'-hexachloro-p-xylene | Full load           | 102                         |

The above formulation without the additive of the present invention gives a tapping efficiency of 83% and fails at 28 pounds on the Almen tester, whereas the formulation with 3% a,a'-hexachloro-p-xylene (M.P. 107°-110° C.) gives a tapping efficiency of 102% and withstands a full load on the Almen E.P. tester.

## EXAMPLE 4

To the following composition:

|                                                                                                                                                      | Percent     |
|------------------------------------------------------------------------------------------------------------------------------------------------------|-------------|
| Naphthenic base mineral oil:                                                                                                                         |             |
| Visc. @ 100° F., SUS                                                                                                                                 | 200-211     |
| Gravity                                                                                                                                              | 19-21       |
| Flash point, ° F.                                                                                                                                    | min. 365    |
| Pour point, ° F.                                                                                                                                     | max. 0      |
| Sulfur, wt. percent                                                                                                                                  | 0.4         |
| Di-tertiary nonyl polysulfide:                                                                                                                       |             |
| Visc.—                                                                                                                                               |             |
| @ 25° C. ca.                                                                                                                                         | 132.5       |
| @ 100° C. ca.                                                                                                                                        | 5.9         |
| Specific gravity                                                                                                                                     | 1.036-1.045 |
| Total sulfur, wt. percent                                                                                                                            | min. 36.5   |
| Active sulfur, wt. percent                                                                                                                           | min. 27.5   |
| Calc. mol. wt.                                                                                                                                       | 414.8       |
| Straight chain fatty acid (a tall oil fatty acid—aver. C <sub>18</sub> carbon chain length alkyl carboxylic acid containing unsaturated components): |             |
| Visc. @ 100° F., SUS                                                                                                                                 | 93          |
| Specific gravity, 25/25                                                                                                                              | 0.9005      |
| Iodine value                                                                                                                                         | 130-140     |
| Saponification No.                                                                                                                                   | 190-195     |
| Flash point, ° F.                                                                                                                                    | 380         |
| Fire point, ° F.                                                                                                                                     | 415         |
| Pour point, ° F.                                                                                                                                     | +37         |

Four percent by weight of a,a'-hexachloro-p-xylene (M.P. 107°-110° C.) is added and the formulation is characterized by the following properties:

|                              |      |
|------------------------------|------|
| Color dil.                   | 3.50 |
| Flash point, ° F.            | 310  |
| Viscosity @ 100° F., SUS     | 177  |
| Pour point, ° F.             | -40  |
| Water content, wt. percent   | Nil  |
| Sap. oil, wt. percent        | 13   |
| Sulfur:                      |      |
| Active, wt. percent          | 1.90 |
| Total, wt. percent           | 3.10 |
| Chlorine:                    |      |
| Active, wt. percent          | 0.17 |
| Total, wt. percent           | 3    |
| 70                           |      |
| Free fatty acid, wt. percent | 8.50 |
| Pounds/gallon                | 7.90 |
| Saponification No.           | 84   |

The Almen and Cornell extreme pressure tests are made on the above formulation containing 4% of the extreme

pressure additive of the present invention and the results are presented in Table IV.

Table IV

| Loads (lbs.) |       | Torque  |       |
|--------------|-------|---------|-------|
| Cornell      | Almen | Cornell | Almen |
| 250          | 2     | 4       | 12    |
| 500          | 4     | 9       | 15    |
| 750          | 6     | 12      | 17    |
| 1,000        | 8     | 16      | 20    |
| 1,250        | 10    | 20      | 23    |
| 1,500        | 12    | 20      | 24    |
| 1,750        | 14    | 21      | 25    |
| 2,000        | 16    | 23      | 25    |
| 2,250        | 18    | 24      | 25    |
| 2,500        | 20    | 26      | 25    |
| 2,750        | 22    | 31      | 26    |
| 3,000        | 24    | 32      | 26    |
| 3,250        | 26    | 50      | 26    |
| 3,500        | 28    | 53      | 26    |
| 3,750        | 30    | 55      | 26    |
| 4,000        | —     | Fail    |       |
| 4,250        | —     |         |       |
| 4,500        | —     |         |       |

Four percent by weight of a,a'-hexachloro-p-xylene in the above formulation gives a torque of 55 at 3750 pounds load on the Cornell tester and a torque of 26 at a jaw load of 30 pounds on the Almen tester.

## EXAMPLE 5

A further example of the effectiveness of the present additive as an extreme pressure agent can readily be seen by the addition of 1% by weight of a,a'-hexachloro-p-xylene (M.P. 107°-110° C.) to the following gear lubricant.

| Naphthenic base mineral oil:                  | Percent   |
|-----------------------------------------------|-----------|
| Initial boiling point, °F.....                | 400       |
| Specific gravity.....                         | 0.7852    |
| Aniline point.....                            | min. 185  |
| Kinematic viscosity—                          |           |
| @ 32° F.....                                  | es. 10.56 |
| @ 100° F.....                                 | es. 3.32  |
| Flash point, °F.....                          | 210 15    |
| Emolein 2957 (di-isoctylazelate):             |           |
| Kinematic visc. @ 100° F.....                 | 12.7      |
| Specific gravity @ 25° C.....                 | 0.9123    |
| Pour point, °F.....                           | -85 41    |
| Emolein 2910 (2-ethylhexyl-pelargonate):..... | 41        |
| Acryloid HF 866 <sup>1</sup> :.....           | 7         |
| Pentachlorophenyl mercapto acetic acid:.....  | 1         |

<sup>1</sup> Viscosity index improver comprising an acrylate polymer produced by Rohm & Haas.

The results from Timken & Cornell extreme pressure tests are given in Table V.

Table V

|                                                                                                                                                                                                                                                                                                                                                                                                      |      |
|------------------------------------------------------------------------------------------------------------------------------------------------------------------------------------------------------------------------------------------------------------------------------------------------------------------------------------------------------------------------------------------------------|------|
| Timken: Pass, lbs. ....                                                                                                                                                                                                                                                                                                                                                                              | 45   |
| Cornell: Failed at load, lbs. ....                                                                                                                                                                                                                                                                                                                                                                   | 4500 |
| The test data in Table V show a 45-lb. Timken value and a high load capacity, e.g., greater than 4500 lbs. before the lubricant fails on the Cornell tester. Also, the above formulation containing the extreme pressure additive of the present invention when subjected to the copper strip corrosion test shows essentially no corrosion of the copper strip after testing for 3 hours at 210° F. |      |
| 55                                                                                                                                                                                                                                                                                                                                                                                                   |      |

It is to be understood that although the invention has been described with specific reference to particular embodiments thereof, it is not to be so limited since changes and alterations therein may be made which are in the full intended scope of this invention as defined by the appended claims.

It is claimed:

1. A lubricating composition consisting essentially of a major amount of oil of lubricating viscosity and a minor amount sufficient to improve extreme pressure characteristics of a compound having the following structural formula:

15



2. The composition of claim 1 wherein the oil of lubricating viscosity is a mineral lubricating oil.

3. The composition of claim 1 wherein the extreme pressure compound is present in amounts between about 0.1 to 10 weight percent.

4. A lubricating oil composition consisting essentially of a major amount of oil of lubricating viscosity and a minor amount sufficient to improve extreme pressure characteristics of bis(trichloromethyl)-p-benzene.

5. The composition of claim 4 wherein the oil of lubricating viscosity is a mineral lubricating oil.

6. The composition of claim 4 wherein the extreme pressure compound is present in an amount between 0.1 to 10% by weight.

7. The composition of claim 4 wherein the extreme pressure compound is present in amounts between about 0.5 to 5 weight percent.

8. A lubricating oil composition consisting essentially of a major amount of oil of lubricating viscosity and a minor amount sufficient to improve extreme pressure characteristics of a mixture of bis(trichloromethyl)-p-benzene and bis(trichloromethyl)-m-benzene.

9. The composition of claim 8 wherein the oil of lubricating viscosity is a mineral lubricating oil.

10. The composition of claim 8 wherein the extreme pressure compound is in an amount between 0.1 to 10% by weight.

11. The composition of claim 8 wherein the extreme pressure compound is present in amounts between about 0.5 to 5 weight percent.

## 50 References Cited by the Examiner

## UNITED STATES PATENTS

|           |       |               |        |
|-----------|-------|---------------|--------|
| 2,261,863 | 11/41 | Whittier      | 252-58 |
| 2,542,286 | 2/51  | Morris et al. | 252-58 |
| 2,558,079 | 6/51  | Gallsworth    | 252-58 |
| 2,971,913 | 2/61  | David et al.  | 252-58 |
| 3,076,039 | 1/63  | Ayers et al.  | 252-58 |

DANIEL E. WYMAN, Primary Examiner.